

Aug. 7, 1923.

1,464,242

A. F. DECKER

PRINTER'S BLANKET

Filed Sept. 16. 1922



Inventor  
Ammiel F. Decker,

By *Hartwell M. Anthony*  
Attorney

Patented Aug. 7, 1923.

1,464,242

# UNITED STATES PATENT OFFICE.

AMMIEL F. DECKER, OF PELHAM, NEW YORK.

## PRINTER'S BLANKET.

Application filed September 18, 1922. Serial No. 588,736.

*To all whom it may concern:*

Be it known that I, AMMIEL F. DECKER, a citizen of the United States, residing at Pelham, in the county of Westchester and State of New York, have invented certain new and useful Improvements in Printers' Blankets, of which the following is a specification.

The present invention relates to improvements in printers' blankets, and more particularly to blankets of the type disclosed in my Patent No. 1,004,385, granted September 26, 1911.

Articles of the character indicated must possess a certain degree of flexibility and resiliency and, in addition, must be capable of resisting the disintegrating action of printer's ink. In my aforesaid patent, I have described a form of blanket comprising a body composition, preferably consisting of ground cork and a binder of resin, linseed oil and gum, faced on opposite sides with fabric or other suitable material. Such blankets, while satisfactory in the initial stages of their use, have, nevertheless, a tendency to soon dry out and lose their resiliency when subjected to use in a dry climate and, in like manner, soon harden and crack or break in a cold climate, so that their period of effective life may, therefore, be substantially reduced by reason of atmospheric and climatic conditions.

It is the object of this invention to overcome the objections stated, by producing a blanket which shall retain its flexibility and resiliency without regard to cold or dryness and which, moreover, shall possess a greater degree of durability and a proportionately longer life.

According to my invention, I employ ground cork as the base of the body composition, as in the earlier form, and I may also use resin and gum. But instead of using linseed oil, which is a drier, with the cork, resin and gum, or with the cork alone, I employ a non-siccative oil, preferably castor oil, which has the effect of preventing the composition from drying out, and which also acts as an emollient. I also use the so-called "nitrated cotton" or other commercial form of nitro-cellulose in a dissolved state, the preferred solvent being ethyl-acetate, though other suitable solvents may, of course, be substituted.

The substances or ingredients mentioned above are intimately mixed together in suit-

able proportions which, however, may be varied at will according to conditions, the cork predominating as will be understood. In this connection, I desire to state that I am aware that both nitrocellulose and castor oil have been used together in the manufacture of printers' blankets, but only as a distinct surfacing layer at one or both sides of the body; whereas I expressly mix both the nitrocellulose and the castor oil with the other ingredients to form the body itself, and because of this thorough admixture of the several ingredients, I prevent the body from cracking or breaking and from becoming hard or dry, or both, while still maintaining its requisite oil- and ink-proof quality.

After the composition has been prepared, it is preferably spread on a strip of suitable facing material, or spread or fed between two such strips or sheets, and is then subjected to sufficient pressure, by passing it between rolls or otherwise, to actually force the composition to enter the meshes, pores or interstices of the facing strip or strips. After this, it is left to set or season, the time required depending upon various factors which in themselves are immaterial to the invention. The facing strip or strips may, and in most cases will, consist of wool, cotton, linen, jute or other fabric; but under certain conditions, strips or sheets made of various other substances such as paper, asbestos, ground slate, metal, rubber, etc., may also be utilized, so that the terms "facing" or "facing sheet" herein employed are expressly used in a generic sense. Moreover, the facing or facings may be suitably coated for ornamental or other purposes, and where special strength is desired, a reinforcement in the form of wire netting or other material may be used and may constitute one of the facings or may be embedded in the body composition; or a coating of adhesive material may be applied to one or both sides of the body composition and a suitable facing affixed thereto.

The accompanying drawing shows, on a greatly enlarged scale, a cross section of a blanket constructed in accordance with the invention, the component parts of the blanket being indicated by appropriate labels.

While the invention, as above disclosed, is primarily a printer's blanket and has been so described, it will be nevertheless appar-

ent that the body composition may be used for the manufacture of artificial shingles and roofing tiles (in which instance the metal reinforcement will preferably be utilized) as well as of boxes, desk tops, trunks, traveling bags, etc., where other reinforcement material would be advisable.

I claim:

1. A printer's blanket or the like, having a body comprising an intimate mixture of ground cork, castor oil and dissolved nitrocellulose.
2. A printer's blanket or the like, having a body comprising a mixture of ground cork, castor oil and dissolved nitrocellulose; said body having a facing applied to at least one face thereof.

3. A printer's blanket or the like, having a body comprising an intimate mixture of ground cork, castor oil and dissolved nitrocellulose; and a facing applied to at least one side of said body and united thereto by pressure so that the body composition penetrates said facing.

4. A printer's blanket or the like, having a body comprising an intimate mixture of ground cork, castor oil and dissolved nitrocellulose; and a sheet of wire netting united to said body by pressure so that the body composition is forced into and fills the meshes of the netting.

In testimony whereof I affix my signature.

AMMIEL F. DECKER.